

Sept. 15, 1931.

W. A. MARRISON

1,823,329

PIEZO ELECTRIC DEVICE

Filed Aug. 26, 1924

Fig.1



Fig.2



Fig.3



Fig.5



Fig.6



Fig.4



Fig.7



Fig.8



Inventor:  
Warren A. Morrison  
by *Edward A. Atty.*

## UNITED STATES PATENT OFFICE

WARREN A. MARRISON, OF EAST ORANGE, NEW JERSEY, ASSIGNOR TO WESTERN ELECTRIC COMPANY, INCORPORATED, OF NEW YORK, N. Y., A CORPORATION OF NEW YORK

## PIEZO ELECTRIC DEVICE

Application filed August 26, 1924. Serial No. 734,189.

This invention relates to piezo electric devices and more particularly to means for increasing the frequency range of such devices.

Heretofore in the design of piezo electric devices used as the frequency control elements in space discharge tube systems, it has been customary to prepare the piezo active element of these devices in the form of a parallelepiped. The piezo crystal is usually arranged between metallic plates upon which alternating electromotive forces are impressed. When so arranged, the piezo element is set into vibration by the action of the electric field between the plates. If the crystal is cut with its longer dimension in the direction of a line perpendicular to one of the natural faces of the mother crystal and the metallic plates are positioned on opposite sides of the crystal on the line of its shorter axis, that is its thickness, the crystal being cut so that this dimension is parallel with an electrical axis, then the crystal will be set into longitudinal vibration in the direction of its longer axis to produce what is known as the transverse effect. Of course, the crystal will also tend to vibrate in the direction of the electric field, that is, as in accordance with what is known as the longitudinal effect although this type of vibration is not of significance in connection with this invention. The natural frequency of the crystal in this mode of vibration depends upon the elastic constant of the substance as well as its density and length. This frequency is given approximately by an equation

$$F = \frac{K}{L}$$

where K is a constant approximately equal to 2,700,000 and L is the length of the crystal in millimeters. It is thus seen that it is comparatively easy to design crystals having natural frequencies within the range of high radio frequencies, for example, from 100 to 2000 kilocycles per sec. A crystal whose frequency is 1,000,000 cycles per sec. would be approximately three millimeters long. Since the frequency of vibration is inversely proportional to the length, this dimension

must be greatly increased to obtain low frequencies. For example, a crystal designed to vibrate at a frequency of 10,000 cycles per second would be approximately 27 centimeters in length. Obviously, it is extremely difficult to obtain quartz or other crystals of these dimensions and even were they readily obtainable, the apparatus employing them would necessarily be cumbersome and difficult to handle.

It is an object of this invention to cause vibration of piezo electric elements at low frequencies.

Another object is to produce transverse that is, flexural vibration of a piezo electric element.

An additional object is to produce piezo electric elements having a ratio of restoring force to mass which is smaller than has heretofore been obtained.

A feature of the invention relates to piezo electric crystals of small dimensions having a shape such that it has a natural frequency lower than has heretofore been obtainable from crystals of equivalent dimensions.

Another feature relates to a piezo electric device having its various elements so arranged that transverse vibration of the vibrating element is produced.

It is found that by cutting piezo electric crystals from quartz in suitable shapes, the ratio of restoring force to mass may be decreased for forces acting in the direction of the longer axis of the crystal. Such crystals are found to have a natural frequency of vibration, in the direction of the longer axis, that is lower than that of crystals cut in the form of parallelepipeds having equivalent dimensions. In addition, it is found that a piezo electric crystal may be set into transverse vibration by properly positioning the metallic plates arranged adjacent to opposite sides of the crystal.

In the drawings, Fig. 1 illustrates the method of cutting a dumb-bell shaped piezo electric crystal in accordance with this invention.

Fig. 2 is a transparent view illustrating the method of cutting the dumb-bell shaped crystal of Fig. 1.

Fig. 3 is an enlarged view of a piezo electric device employing a dumb-bell shaped crystal.

Fig. 4 is an end view of the device shown in Fig. 3.

Fig. 5 illustrates a piezo electric device arranged for transverse vibration of the crystal.

Fig. 6 illustrates the mode of vibration of the crystal of Fig. 5.

Fig. 7 is an end view of the piezo electric device of Fig. 5.

Fig. 8 illustrates a modification of the device shown in Fig. 5.

In Fig. 1, a dumb-bell shaped crystal 11 is shown in the position with respect to the mother crystal 12 from which it is cut. Lines 10 represent the six natural faces of the crystal 12. The dumb-bell shaped crystal 11 is preferably so cut from the mother crystal 12 that its longer axis is perpendicular to one of the natural faces of the original crystal as illustrated.

In Fig. 2 a transparent side view of the crystal 12 of Fig. 1 is shown. The dumb-bell shaped crystal 11 is illustrated in the position from which it is cut. The dotted lines 1 and 2 represent the longer and shorter axes respectively, of this crystal.

In Fig. 3, the dumb-bell shaped crystal 11 is shown positioned between the metallic plates 13.

An end view of the piezo electric device as shown in Fig. 3 is illustrated in Fig. 4 in which the position of the plates 13 is more clearly shown. When a source of alternating electromotive force is applied to the terminals 14, the crystal 11 is set in longitudinal vibration in the direction of the dotted axis 1 of Fig. 3. By virtue of the enlarged ends provided on the crystal 11, the mass of the crystal is increased without substantially increasing the restoring force. It is thus seen that the ratio of restoring force to mass is correspondingly reduced and as a result the natural frequency of the vibration of the crystal 11 is also reduced. The following table gives the natural frequency of vibration for several samples of crystals of dumb-bell shape having a length of 5.6 cm., a width at the end sections in the direction of axis 2 of Fig. 2 of 1.2 cm. and a thickness of .5 cm. The column headed "A" is the width of the reduced portion in the direction of axis 2 in centimeters.

|    |     | Natural frequency |
|----|-----|-------------------|
| 60 | .98 | 44,675            |
|    | .73 | 39,500            |
|    | .54 | 37,580            |
|    | .38 | 33,280            |
|    | .29 | 28,960            |
|    | .18 | 24,960            |

In Figs. 5 and 7, a piezo electric device arranged to produce low frequency vibra-

tions by another method is illustrated. In this device, the crystal 11 is cut in the form of a parallelepiped. The plates 13 are positioned along one edge at opposite sides of the crystal 11. With this arrangement of the plates the crystal 11 is set into vibration, upon the application of alternating electromotive forces to the plates 13, in the manner illustrated by the curves of Fig. 6. This mode of vibration is produced by virtue of the fact that the portion of the crystal directly opposite the plates 13 undergoes contraction and expansion whereas the portion of the crystal away from the plates 13 has substantially no strains produced therein. The result is a transverse flexing of the crystal 11. It is well known that in one mode a free-free bar vibrates about two nodes such as nodes 15 illustrated in Fig. 6, at approximately 0.224 of the length of the bar from its ends. The natural frequency of the bar or crystal in this mode of vibration can be accurately determined from the elastic constant, the density, and the dimensions of the bar. See Barton's textbook on Sound, 1914 edition, pages 280 to 288 inclusive published by MacMillan & Company, Ltd., St. Martin Street, London, wherein on page 281 the frequency  $N$  is shown equal to

$$m^2 \frac{K}{2\pi l^2} \sqrt{\frac{q}{p}}$$

in which  $N$  is a quantity, the value of which is to be determined by further calculations not essential to the present disclosure,  $K$  is the radius of gyration,  $l$  is the length of the bar,  $q$  is Young's modulus of elasticity and  $p$  is the density of the material.

The crystal element 11 is preferably cut from the mother crystal as already explained with respect to the crystal of Fig. 3 having its longer axis perpendicular to one of the natural faces of the mother crystal as shown in Figs. 1 and 2.

In Fig. 8 a modification of the piezo electric device shown in Fig. 5 is illustrated wherein additional plates 13' are provided for utilizing both sections of the crystal. By means of the device illustrated in this figure, a greater response of the crystal may be obtained for a given impressed alternating electromotive force wave. If desired, an electromotive force of frequency corresponding to the natural frequency of the crystal may be applied to the plates 13 and a corresponding electromotive force having its frequency determined solely by the natural frequency of the crystal may be obtained from plates 13'.

Piezo electric devices constructed in accordance with this invention may be applied as frequency control elements in space discharge tube systems for frequencies within the audible range.

Although the invention has been described in connection with certain specific embodiments, the principles disclosed are applicable to other practical arrangements and the invention is therefore to be limited only as indicated by the scope of the appended claims.

What is claimed is:

1. A piezo electric device comprising a vibratory element of piezo electric material and conducting plates, subjected to electromotive forces, placed adjacent corresponding portions of opposite sides of said element parallel to its longer axis and unsymmetrically with respect to said axis whereby said element tends to vibrate transversely.
2. A piezo electric device comprising a vibratory element of quartz material, and conducting plates, subjected to electromotive forces, placed adjacent corresponding portions of opposite sides of said element parallel to its longer axis and unsymmetrically with respect to said axis whereby said element tends to vibrate transversely.
3. A piezo electric device comprising a quartz crystal body in the form of a parallelepiped and conducting plates, subjected to electromotive forces, placed adjacent corresponding portions of opposite sides of said crystal parallel to its longer axis and unsymmetrically with respect to said axis whereby said crystal tends to vibrate transversely.
4. A piezo electric device comprising a parallelepiped of quartz material having one dimension greater than another, and conducting plates, subjected to electromotive forces, placed adjacent corresponding portions of opposite sides of said parallelepiped parallel to its longer dimension and unsymmetrically with respect to the axes of the respective sides whereby said parallelepiped tends to vibrate transversely at a lower frequency than can be obtained by longitudinal vibration in the direction of said longer dimension.
5. A piezo electric device comprising a plurality of pairs of conducting plates subjected to electromotive forces from a single source, and a parallelepiped of quartz material therebetween, each of said pairs of plates being placed adjacent corresponding portions of opposite sides of said quartz parallelepiped parallel to its longer axis and unsymmetrically with respect to said axis, whereby said parallelepiped tends to vibrate transversely of its longer axis.
6. The method of operating a piezo electric oscillator comprising a single homogeneous quartz piezo electric element, which consists of simultaneously producing mechanical stresses of opposite sense in different parts of said element.
7. The method of operating a piezo elec-

tric quartz crystal which comprises simultaneously impressing differences of potential of relatively opposite sign across different parts of a crystal whereby there is induced a compressive stress in one part of said crystal and a tensile stress in another part of said crystal.

8. The method of operating a piezo electric crystal having a conformation of a rectangular parallelepiped, the long dimension of which is perpendicular to a face of the natural crystal which comprises simultaneously impressing differences of potential of relatively opposite sign across different parts of the crystal and so as to electrostatically stress the crystal in a direction parallel with a side of the natural crystal whereby there is induced a compressive stress in one part of said crystal and a tensile stress in another part of said crystal.

In witness whereof, I hereunto subscribe my name this 22nd day of August A. D., 1924.

WARREN A. MARRISON.

70

75

80

85

90

95

100

105

110

115

120

125